

Feb. 12, 1946.

L. S. RENZONI

2,394,874

ELECTRO-REFINING OF NICKEL

Filed Jan. 15, 1943

9 Sheets-Sheet 1

FIG. 1.



INVENTOR.  
LOUIS S. RENZONI

BY

C. Ar. Weller  
ATTORNEY

Feb. 12, 1946.

L. S. RENZONI

2,394,874

ELECTRO-REFINING OF NICKEL

Filed Jan. 15, 1943

9 Sheets-Sheet 2

Fig. 2.



INVENTOR.

LOUIS S. RENZONI

BY

*A. Dr. Miller*

ATTORNEY

Feb. 12, 1946.

L. S. RENZONI

2,394,874

ELECTRO-REFINING OF NICKEL

Filed Jan. 15, 1943

9 Sheets-Sheet 3

Fig. 3.



INVENTOR

LOUIS S. RENZONI

BY *A. P. Deller*  
ATTORNEY

Feb. 12, 1946.

L. S. RENZONI

2,394,874

ELECTRO-REFINING OF NICKEL

Filed Jan. 15, 1943

9 Sheets-Sheet 4

FIG. 4.



INVENTOR.  
LOUIS S. RENZONI  
BY

*A. P. Weller*  
ATTORNEY

Feb. 12, 1946.

L. S. RENZONI

2,394,874

ELECTRO-REFINING OF NICKEL

Filed Jan. 15, 1943

9 Sheets-Sheet 5

Fig. 5.



pH 5.4 TEMP. 135°F

INVENTOR.

LOUIS S. RENZONI

BY

A. Dr. Weller  
ATTORNEY

Feb. 12, 1946.

L. S. RENZONI

2,394,874

ELECTRO-REFINING OF NICKEL

Filed Jan. 15, 1943

9 Sheets-Sheet 6

FIG. 6.



INVENTOR.

LOUIS S. RENZONI

BY

*A. P. Weller*  
ATTORNEY

Feb. 12, 1946.

L. S. RENZONI

2,394,874

ELECTRO-REFINING OF NICKEL

Filed Jan. 15, 1943

9 Sheets-Sheet 7



Feb. 12, 1946.

L. S. RENZONI

2,394,874

ELECTRO-REFINING OF NICKEL

Filed Jan. 15, 1943

9 Sheets-Sheet 8



Feb. 12, 1946.

L. S. RENZONI

2,394,874

ELECTRO-REFINING OF NICKEL

Filed Jan. 15, 1943

9 Sheets-Sheet 9

*FIG. 8.*



*FIG. 9.*



INVENTOR  
LOUIS S. RENZONI  
BY *A. P. Deller*  
ATTORNEY



ification of the impure anolyte and for the electro-deposition of cathode nickel or electro-nickel from purified electrolyte in accordance with the principles of the present invention;

Fig. 8 is a photomicrograph taken at 500 magnifications of electro-nickel produced in an all-sulfate ion bath at 12 amperes per square foot; and

Fig. 9 is a photomicrograph taken at 500 magnifications of electro-nickel produced in a sulfate-chloride electrolyte at 16 amperes per square foot.

Briefly stated, the electro-refining of nickel involves the production of impure nickel anodes which are cast in any suitable manner and generally have a nickel content of about 90% to about 96%. Dependent upon the source of the nickel from which the impure nickel anodes are produced, such anodes will contain greater or lesser amounts of the impurities present in the ore. Thus, for example, in one industrial operation, the impure nickel anodes contain about 94% to about 96% of nickel, about 2.5% to about 3.5% of copper, about 0.7% to about 0.9% of cobalt, about 0.5% to about 1.0% of iron, about 0.002% to about 0.004% of lead, about 0.05% to about 0.07% of arsenic and about 0.5% to about 0.8% of sulfur.

The electro-refining of nickel involves solution of the metallic constituents of the impure anode in the anolyte followed by purification of the anolyte to remove iron, copper, cobalt, lead, arsenic, etc. to obtain a purified electrolyte from which electro-nickel can be produced.

Electrolytic nickel produced in the all-sulfate electrolyte has the following composition:

| Composition  | Per cent                    |
|--------------|-----------------------------|
| Nickel.....  | About 99.18 to about 99.29. |
| Cobalt.....  | About 0.80 to about 0.70.   |
| Copper.....  | About 0.005 to about 0.003. |
| Iron.....    | About 0.008 to about 0.005. |
| Lead.....    | About 0.004 to about 0.002. |
| Arsenic..... | About 0.003 to about 0.002. |

The general features of the electrolytic cell preferably employed in conjunction with the Hybinette bag are described more or less in detail, together with the process employed in conjunction therewith, in the Hybinette U. S. Patent No. 805,969. In the prior art all-sulfate process, the electro-refining of nickel is generally and preferably carried out employing Hybinette bags. As those skilled in the art know, the Hybinette bag generally comprises a wooden frame of spruce or the like covered with a canvas of such weight that a slight hydrostatic pressure maintained on the cathode side of the canvas substantially prevents the migration of copper, cobalt, nickel, iron and similar cations from the impure electrolyte through the canvas diaphragm into the purified electrolyte present as a catholyte in the cathode compartment of the cell.

As clearly set forth in U. S. Patent No. 805,969, a hydrostatic pressure is maintained in the cathode compartment and impure anolyte withdrawn from the anode compartment continuously. The impure anolyte is first subjected to purification to remove copper and, in the all-sulfate ion electrolyte, the copper is removed by cementation through addition of nickel, preferably in the form of freshly reduced nickel powder, before the iron, lead and arsenic are removed. After the copper has been removed by cementation, the iron, lead and arsenic are then removed. When desired,

the cobalt is removed in the all-sulfate ion electrolyte by the addition of nickel, preferably in the form of an oxide or hydrated oxide prepared outside the electrolyte system by the action of a strong oxidizing agent upon nickelous hydrate, whereby the nickel goes into solution and the cobalt is precipitated. This, however, is a difficult and costly operation. In order to derive the advantages of lower tank voltage, higher anode efficiency, lower steam consumption, better purification of impure anolyte, the production of a more highly purified electro-nickel, and other advantages of the present invention, it was found that the sequence of steps for the purification of the impure anolyte which had provided satisfactory results when employed in conjunction with the all-sulfate-ion electrolyte was ineffective when employed in conjunction with the novel electrolyte of the present invention containing chloride ions equivalent to up to about 50 grams of sodium chloride per liter.

In the operation of the all-sulfate process, anode efficiency is lower than cathode efficiency which results in anolyte flowing from the plating tanks at pH 3.0 to pH 3.2. This value is too low for iron hydrolysis and must be raised to a minimum of pH 5.0 before attempting iron precipitation. The pH rise is brought about by carrying out copper cementation before iron hydrolysis. The nickel powder functions in cementing copper and in neutralizing excess acid. Thus, in one operation using anodes containing 2.65% copper, the cementation of 100 pounds of copper requires the dissolution of 173 pounds of reduced nickel powder. Of this amount, 92 pounds are required for cementing copper and 81 pounds for neutralizing acid. In the sulfate-chloride process, anode efficiency is practically equal to cathode efficiency and anolyte pH is 4.6. This allows for the removal of iron in the presence of cupric ions. During copper cementation the amount of excess acid present is small. Thus, in the operation using anodes containing 2.65% copper, the cementation of 100 pounds of copper requires 133 pounds of nickel powder, of which 41 pounds are consumed for acid neutralization. The operation of the sulfate-chloride process, therefore, shows a clear saving in nickel powder consumed for copper cementation.

In order that those skilled in the art may have a clearer understanding of the present invention, the process will first be described in conjunction with the simplified flow sheets, Figures 1 to 6, and then the process will be described in conjunction with the drawings, Figs. 7 and 7a.

The refining of nickel-containing material by electro-deposition of nickel from a purified electrolyte involves the use of a number of electrolytic cells employing a diaphragm to separate impure anolyte from the catholyte. The number of cells required is, of course, dependent upon the amount of nickel to be electro-deposited in a unit of time, most of the cells being operated with a soluble anode while a few of the cells are operated employing insoluble anodes. The soluble anodes are obtained by casting or otherwise forming from impure metallic material containing a relatively high percentage of nickel, but also containing so much of the impurities, copper, iron, cobalt, lead, arsenic and sulfur, that the impure anodes are not acceptable, per se, to the trade as pure nickel. The impure anodes are immersed in the anode compartment of the diaphragm cell in contact with lean anolyte obtained from previous operations, i. e., catholyte, the nickel content of

which has been suitably lowered by electro-deposition of nickel, because the density of the electric current and the anions present in the lean anolyte, the soluble impure anodes are more or less completely dissolved in the lean anolyte with the production of an impure anolyte containing practically all of the nickel and the base metals, copper, cobalt, iron, lead and arsenic. The precious metals, gold, platinum and other metals of the platinum metal group together with sulfides of copper and nickel, present in the soluble impure anodes, remain on the more or less completely dissolved impure anodes as anode slimes in quantities dependent upon previous operations and the source of the nickel.

In Figure 1 there is provided a simplified flow sheet illustrating in a diagrammatic manner the removal of iron, arsenic and lead, together with the copper cementation removal of copper as carried out in the present process. Preferably, conditions of temperature, pH and other conditions are as indicated in the flow sheet. As those skilled in the art will understand, the impure electrolyte is first treated at a temperature of about 135° F. with air to practically completely oxidize the copper from the cuprous to the cupric state and the iron from the ferrous to the ferric state. In the presence of cupric ions, this reaction takes place rapidly at temperatures as low as 100° F. Upon oxidation of iron to the ferric state, hydrolysis takes place and the iron is completely hydrolyzed and precipitated as ferric hydroxide. By maintaining the proper ratio of cuprous ions to ferrous ions in the impure electrolyte, the hydrolysis of iron takes place substantially without change in the pH of the solution. Thus, the acid released upon hydrolysis of the ferric ion is neutralized by the oxidation of the cuprous ion, and no alkali is required to maintain the electrolyte pH at the value required for complete iron hydrolysis. Following the substantially complete precipitation of iron, the electrolyte plus suspended ferric hydroxide is treated with molecular chlorine from the insoluble anodes. Under these conditions, the arsenic is oxidized to the pentavalent state, in which condition they are precipitated by the action of the suspended ferric hydroxide and removed. The fluid portion of the electrolyte is then treated with nickel powder and copper is thrown out of the solution as cement-copper. The reaction proceeds at 135° F. and no external heat is required. The cement-copper is separated from the fluid portion which then has a pH of 5.4. Thereafter, the pH of the solution is lowered to about pH 4.5 by the addition of any suitable acid, preferably, sulfuric acid, or electrolyte flowing from the insoluble anode tanks. The purified electrolyte, having a temperature of about 135° F. and a pH of about 4.0 to about 5.0, is then introduced into the cathode compartments of the electro-refining cells having soluble and insoluble anodes. In the cathode compartments of the electro-refining cells having soluble or insoluble anodes, approximately 25% of the nickel is removed. At soluble anodes, this quantity of nickel is replaced by an equivalent amount of the cations nickel, copper and iron. Since, however, in the normal operation of the process, copper enters the solution in the cuprous state and is later cemented from the cupric state, the nickel content of the purified electrolyte will progressively increase. In order to maintain the nickel content at a constant level, it is necessary to provide a suitable number of electro-refining cells having insoluble

anodes. In such cells, 25% of the nickel is removed from the catholyte, but no metals are dissolved at the anodes. Instead chlorine and hydroxyl anions are discharged at about 75% and 25% current efficiency, respectively, to produce a mixed gas consisting of molecular chlorine and oxygen which is collected and distributed throughout the process as indicated. The fluid portion of the anolyte flowing from the insoluble anode cells contains approximately 75% of the nickel contained in purified electrolyte and has an acid content equivalent to 4 to 6 grams per liter sulfuric acid and a dissolved chlorine content of 0.2 to 0.4 gram per liter. This acid solution is used for the treatment of primary iron slimes in the event that they contain little or no cobalt. If the primary iron slimes is to be treated for cobalt recovery, the acid solution is then used for pH correction of the purified electrolyte flowing from the copper filter presses to the electro-refining cells. After treatment with the anolyte from the insoluble anodes plus sulfuric acid, if required, treated slimes are obtained together with a solution containing the nickel of the primary slimes. This solution is returned to the main stream of impure anolyte.

A simplified illustration of the removal of iron, arsenic and lead from the impure anolyte is provided in Fig. 2. It would appear that the cupric copper present in the impure anolyte oxidizes the ferrous ions always present to ferric ions and the ferric salts thus produced hydrolyze to form ferric hydroxide. The air or other oxygen-containing gases which are passed through the solution oxidize the cuprous ions to cupric ions, making possible the further oxidation of further amounts of ferrous salts. It is believed that this reaction may be represented by the following equation:

$$4\text{FeCl}_2 + 4\text{CuCl}_2 + 3\text{O}_2 + 6\text{H}_2\text{O} \rightarrow 4\text{Fe}(\text{OH})_3 + 8\text{CuCl}_2$$

The purification of primary iron slimes containing cobalt and the recovery of cobalt is illustrated in the simplified diagrammatic flow sheet, Fig. 3. Primary slimes containing cobalt are treated preferably with sulfur dioxide and sulfuric acid, although any reducing agent capable of reducing ferric iron to ferrous iron may be employed. Under these conditions, all of the cobalt, nickel and 15% to 20% of the iron are reduced from the oxidized, relatively acid insoluble states to the readily soluble reduced states. With sulfur dioxide, copper forms the relatively insoluble cuprous sulfite which may be removed by filtration at this stage, but which may also be retained in suspension and re-dissolved in the next step. Complete solution of all the constituents with the exception of cuprous sulfite takes place at pH 2.0. Iron may then be removed from the cobalt, nickel, iron solution having cuprous sulfite suspended therein by further additions of primary iron slimes. By so doing, the ferrous ion is oxidized to the ferric state and the cuprous sulfite to cupric sulfate by the action of nickellic and cobaltic hydrates which are in turn reduced and enter the solution. The dissolution of the nickellic and cobaltic hydrates also neutralizes sufficient acid to allow for complete iron hydrolysis. The reactions involved in the oxidation and hydrolysis of iron may be expressed as follows:

Reduced II base base ferric eff. when purified  
-> FeSO<sub>4</sub> + Co(OH)<sub>3</sub> → CoSO<sub>4</sub> + Fe(OH)<sub>3</sub> [Addition  
bentonite] Cu<sub>2</sub>SO<sub>3</sub> + 4Co(OH)<sub>3</sub> + 5H<sub>2</sub>SO<sub>4</sub> → [addition  
of eddies like] 4CoSO<sub>4</sub> + 2CuSO<sub>4</sub> + 11H<sub>2</sub>O yielding as  
moist eff as moist since eff is added eff however

Thus, an iron slime, which may be called secondary iron slime, is formed and is separated from the fluids containing nickel, cobalt and copper in the form of soluble salts. The secondary iron slimes contain about 40% iron and small amounts of copper, cobalt and nickel which may be treated in any suitable manner for the recovery of copper, cobalt and nickel therein contained. The fluid portion containing the nickel, cobalt and copper as sulfates, preferably, is treated with nickel powder at a pH of about 5.2 to precipitate the copper as cement-copper and the cement-copper is removed in any suitable manner such as, for example, by a filter press. The fluid portion containing the nickel and cobalt as sulfates is treated with an alkaline oxidizing agent to preferentially oxidize and hydrolyze the cobalt. Preferably, an alkaline solution of sodium hypochlorite is employed as the oxidizing and precipitating agent. The cobalt is precipitated as a hydrated oxide or hydroxide containing from 53 to 55% cobalt, 2 to 4% nickel, and traces of copper and iron. The precipitate is allowed to settle and the supernatant nickel solution, now containing only approximately 0.2 gram per liter cobalt is removed by decantation. The nickel values are recovered from this solution by precipitation as basic nickel carbonate which is then collected in a filter press, washed, resuspended in water and added to oxidation tank No. 3 of the nickel electrolyte purification system to supply a portion of the alkali required for cobalt hydrolysis. The first cobalt precipitate is resuspended in water and redissolved by the addition of sulfur dioxide and sulfuric acid. The resulting solution, containing approximately 30 grams per liter cobalt, and 1 to 2 grams per liter nickel is again treated with an alkaline sodium hypochlorite solution and the cobalt is again precipitated. The second cobalt precipitate contains from 55 to 57% cobalt, from 0.4 to 0.6% nickel and traces of copper and iron. The fluid portion from the second cobalt precipitation contains approximately 0.5 gram per liter nickel and approximately 0.2 gram per liter cobalt and is used for washing the first cobalt precipitate. It is believed that the reduction of the iron from the ferric state to the ferrous state and the oxidation of the reduced iron to the ferric state followed by hydrolysis and precipitation as ferric hydroxide is illustrated by the following equation:



In Fig. 4 there is provided in a more or less diagrammatic manner a simplified flow sheet illustrative of the removal of arsenic and lead. After the oxidation and precipitation of the iron has been completed, chlorine is introduced into the impure electrolyte and the arsenic, lead and cobalt oxidized to the higher states of oxidation. Instead of the chlorine, other oxidizing agents, such as hydrogen peroxide, persulfates, and the like, could be employed, but it is preferred to use chlorine in view of the fact that an ample supply is available at the insoluble anode of the electro-refining cells. The arsenic, lead, and, if desired, cobalt are oxidized. The arsenic and lead precipitate, together with the iron, may be removed as primary iron slimes. When it is desirable to remove the cobalt at the same time as the iron,

arsenic and lead are removed, it is necessary to maintain the solution at a pH of about 4.0 to about 5.0 and preferably at a pH of about 4.5 and to augment the chlorine produced at the insoluble anodes with chlorine from an outside source. In order to establish and maintain the desirable pH for precipitation of cobalt, an alkali is added, preferably basic nickel carbonate, to the impure electrolyte in sufficient quantity to maintain a pH between the aforesaid limits.

The flow sheet of Fig. 5 is illustrative in a more or less diagrammatic manner in a simplified way of the removal of copper from the partially purified electrolyte by cementation. The partially purified anolyte is introduced into the first cementation tank into which likewise are introduced the solids from the settler or Dorr tank. The contents of the first cementation tank then pass to the second cementation tank from which the cement-copper is removed. This cement-copper contains about 80% to 90% copper and about 7% to 10% nickel and is further treated for the separation and recovery of the values contained therein. The impure electrolyte passes from cementation tank 2 (corresponding to tank 14 of Fig. 7) to cementation tank 3 (corresponding to tank 15 of Fig. 7) where nickel is added at intervals, preferably, and in amounts sufficient to maintain the copper content of the overflow from the settling tank (or Dorr tank 18 as shown in Fig. 7) below a particular value of about 0.01 to about 0.02 gram per liter. Cement-copper containing some nickel is likewise introduced into cementation tank No. 3 (corresponding to tank 15 of Fig. 7). The precipitated copper and the partially purified electrolyte then pass to two additional copper cementation tanks to allow sufficient time for the reaction, and thence to a settling tank or Dorr tank where the solids are removed and conveyed to the first cementation tank and the overflow or solution of partially purified electrolyte passes to cementation tank No. 6 (corresponding to tank 19 of Fig. 7) where the nickel powder necessary to remove substantially all of the residual copper is added. To provide time for the reaction to reach completion, the contents of cementation tank No. 6 (corresponding to tank 19 of Fig. 7) are conveyed to cementation tank No. 7 (corresponding to tank 20 of Fig. 7) and then to a suitable means for removing cement-copper from the solution, such as filter press 22 (Fig. 7). The filter press has been found to be satisfactory for this purpose. The filter cake comprises the cement-copper and unused nickel powder and is returned to cementation tank No. 3. When the cobalt has been removed with the iron, the filtrate contains about 0.001 gram to about 0.01 gram, preferably about 0.005 gram per liter of cobalt and is of sufficient purity to be electrolyzed in the electro-refining cells. When the cobalt has not been removed in the iron removal unit, the filtrate is passed to the cobalt removal system. The reaction by which the copper is cemented out of solution is believed to be illustrated by the following equation.



pH \_\_\_\_\_ 4.2 to 5.4  
Temperature \_\_\_\_\_ °F \_\_\_\_\_ 135

During the cementation of the copper, it is preferable to maintain the temperature of the electrolyte at about 135° F. and to allow the pH to rise from about 4.2 to about 5.4. However, a temperature between about 120° F. and about 160° F.

and a pH within the range of about 4.0 to about 5.5 are also satisfactory.

In the event that the removal of iron, arsenic and lead is carried out under such conditions that the cobalt is not precipitated, it is necessary to remove the cobalt after the iron, arsenic, lead and copper have been removed from the impure anolyte. Such an anolyte may be termed partially purified electrolyte. The removal of cobalt is illustrated in a simplified and more or less diagrammatic manner in Fig. 6. The partially purified electrolyte containing about 0.0002 to about 0.0005 gram per liter of copper and about 0.12 gram per liter to about 0.15 gram per liter of cobalt is conveyed to a reaction tank into which molecular chlorine and nickel carbonate are introduced in sufficient quantities to precipitate cobalt to yield a purified electrolyte containing a residual concentration of 0.001 gram per liter to 0.01 gram per liter cobalt. The cobalt precipitates as an oxide or hydrated oxide at a pH of about 4.5 to about 5.0. The suspension is treated to remove the cobalt precipitate in any suitable manner and preferably with a filter press to obtain a cobalt precipitate containing about 18% to about 20% cobalt, about 25% to about 30% nickel, about 0.005% to about 0.01% iron, which is then treated preferably in accordance with the process illustrated in Fig. 3 for the recovery of the cobalt. The filtrate which is now the purified electrolyte for direct introduction into the cathode compartments of the electro-refining cells contains about 0.001 to about 0.01 gram per liter of cobalt, about 0.0002 gram per liter to about 0.0005 gram per liter of copper, about 0.0001 gram per liter of arsenic, about 0.0001 gram per liter of lead, and about 0.0001 gram per liter of iron. It is believed that the reaction to precipitate cobalt in the aforesaid described manner is illustrated by the following equation:



The impure anolyte is removed from the anode compartments 1 (Fig. 7) and transferred by means of conduit 2 to a holding tank 3. The impure anolyte as withdrawn from the anode compartments has a temperature of about 130° F. to about 140° F., a pH of the order of pH 4.6 and contains about 0.25 gram per liter to about 0.35 gram per liter of copper, about 0.07 gram per liter to about 0.10 gram per liter of iron, about 0.0002 gram per liter to about 0.0004 gram per liter of lead, about 0.004 gram per liter to about 0.006 gram per liter of arsenic, and about 0.12 gram per liter to about 0.15 gram per liter of cobalt. The impure electrolyte in holding tank 3 is then conveyed in any suitable manner, for example by means of pump 4 and conduit 5, to the unit for removal of iron, arsenic and lead which comprises four or more containers, such as tanks 6, 7, 8 and 9, connected in series. The contents of tanks 6, 7 and 8 are agitated, preferably by air introduced therein by means of conduit 28. The removal of iron, arsenic and lead is based upon the oxidation of the iron, arsenic and lead and the precipitation of these materials as oxides or hydrated oxides or hydroxides or as insoluble iron and lead compounds of arsenic. In order to precipitate the arsenic and lead, it was found necessary to introduce an oxidizing agent, such as hydrogen peroxide, persulfates, sulfur dioxide and air or chlorine into the reaction mixture after the iron had been oxidized and precipitated.

This is quite contrary to usual practice when purifying an impure all sulfate-ion anolyte.

In the impure anolyte, a portion of the copper is present as cupric ions. The iron is oxidized at the expense of the cupric ions and the cupric ions reoxidized by air passed into the oxidation tanks. The oxidized iron then hydrolyzes and precipitates as the hydroxide. The pH change during the oxidation of the iron and the precipitation thereof is very slight, being equivalent to a drop from pH 4.6 to pH 4.5. It would appear that the successful oxidation of the iron and precipitation thereof is dependent upon the ratio of cuprous copper to the total iron present in the solution. Under normal operating conditions, this ratio is such that practically no pH change occurs. Under these conditions, iron oxidation and hydrolysis takes place rapidly and at low temperatures without requiring the addition of alkali and the reaction is complete in oxidation tank 7. The contents of tank 7 are transferred to tank 8 and thoroughly mixed by circulation through pump 10 or by other suitable means and an oxidizing agent, preferably chlorine, is introduced by suitable means 54 for the oxidation of arsenic from the trivalent to the pentavalent stage and for the oxidation of lead from the bivalent to the tetravalent stage. Preferably, the chlorine is obtained from the anode compartments of the electro-refining cells 84 having insoluble anodes. At the same time, more or less of the cobalt present in the impure anolyte is likewise oxidized and under proper conditions can be removed, together with the iron, lead, arsenic and some copper. However, when desirable, the removal of iron, lead and arsenic can be so controlled as to substantially eliminate the removal of cobalt at this place in the purification system and the cobalt can be removed at a later stage in greater purity. The oxidation of the iron, lead and arsenic is substantially completed in oxidation tank 8 and oxidation tank 9 is only provided to insure the completion of the reaction. The arsenic content of the electrolyte is lowered from about 0.005 gram per liter to about 0.0001 gram per liter after passage through oxidizing tank 8. The iron, arsenic and lead precipitates, together with any cobalt and copper which are precipitated, are removed as primary slimes in any suitable manner, preferably by any suitable means 11 to a filter press 12. The filter cake (primary iron slimes) is treated for the recovery of cobalt as hereinafter described in conjunction with Figs. 3 and 7a, while the filtrate is further treated to remove copper and traces of cobalt.

Copper is removed by cementation after the removal of iron, lead and arsenic has been completed and is carried out in the copper cementation system as illustrated in a diagrammatic manner in Fig. 7 and in the simplified flow-sheet Fig. 5. The copper cementation unit includes seven or more cementation and holding tanks 13, 14, 15, 16, 17, 19 and 20 and a settler 18, such as a Dorr tank. The filtrate from the primary slimes separation (accomplished in filter press 12) is introduced through conduit 21 into cementation tank 13. Freshly reduced nickel powder is introduced into cementation tank 19 into which the overflow of the settler or "Dorr" tank 18 is introduced. The effluent from cementation tank 20 passes to a filter press 22 or other means of separating solids from liquids in which the cement copper, together with some nickel, is separated from the partially purified electrolyte. The solids from this separation containing an appre-

ciable amount of nickel are introduced into cementation tank 15 by suitable means 23. Additional nickel powder, together with the filter cake from press 22 is likewise introduced into cementation tank 15 in amounts sufficient to maintain the copper content of the overflow from the settler tank not greater than about 0.02 gram per liter. The solids settling out in the settler or Dorr tank are returned to the first cementation tank 13 of the system by suitable means, such as pump 24 and conduit 25, and the cement copper is removed from cementation tank 14 in any suitable manner.

Dependent upon the conditions existing in the unit for the removal of iron, arsenic and lead, the electrolyte flowing from the copper cementation system is more or less purified of cobalt. In the event that sufficient cobalt has been removed in the iron, lead, arsenic system, the electrolyte is sufficiently purified to be introduced directly into the cathode compartments 31 of the electrolytic cells by means of conduit 26. On the other hand, if sufficient cobalt has not been removed, the electrolyte flowing from the copper cementation unit, filter press or the like 22, is transferred by means of conduit 27 to tank 28 and treated with chlorine plus nickel carbonate to precipitate the cobalt as a cobaltic hydrate. The cobalt precipitated is separated from the electrolyte by suitable means, such as filter press 29 to which the contents of tank 28 are transferred by suitable means 30, and the purified electrolyte is then introduced into the cathode compartments 31 of the electro-refining cells by means of conduits 32 and 26. The electrolyte, when introduced into the cathode compartments of the refining cells, does not contain greater quantities of cobalt, copper, arsenic, iron and lead than as follows:

| Constituents | Grams per liter                    |
|--------------|------------------------------------|
| Cobalt.....  | From about 0.001 to about 0.01.    |
| Copper.....  | From about 0.0002 to about 0.0005. |
| Arsenic..... | About 0.0001.                      |
| Iron.....    | About 0.0001.                      |
| Lead.....    | About 0.0001.                      |

It is preferred to maintain the electrolyte at a temperature between about 130° F. and about 140° F. during purification and electro-deposition. The pH of the catholyte during electro-deposition is preferably maintained at about 4.0 to about 5.0.

It is desirable to recover the cobalt whether precipitated with the iron, arsenic and lead or removed separately. Furthermore, in view of the fact that an appreciable amount of nickel is precipitated with the iron, lead and arsenic of the primary slimes, it is desirable to further treat the primary slimes, whether they contain cobalt or not, to recover the nickel contained therein and to reintroduce the nickel so recovered into the electro-refining system.

In the event that the primary slimes contain cobalt in amounts greater than 5% to 6%, the treatment of the primary slimes differs from the treatment to which the primary slimes are subjected when the primary slimes contain less than 5% cobalt. When the primary slimes contain more than 5% to 6% cobalt, the primary slimes from filter press 12 are introduced into container 33 by suitable means such as conduit 34 and suspended therein in water (Fig. 7a). Sulfur dioxide, or any other suitable reducing agent is introduced and the reduction reaction is allowed

to proceed until all of the nickel, cobalt and copper, and from about 5% to about 10% of the iron are reduced from the oxidized to the reduced states. When sulfur dioxide is used as the reducing agent, the end point of the reaction is reached when the pH value of the suspension has been reduced to pH 4.3 to pH 4.5. Any suitable acid, preferably sulfuric acid, is then introduced in an amount required to reduce the pH to 1.5 to 2.0 at which value the slime is completely dissolved. During the reaction, the temperature in container 33 rises from about 80° F. to about 120° F. and no external heat is required. When the reaction is completed, the cobalt and nickel compounds and preferably a part of the iron and copper compounds of the primary slimes have been reduced and brought into solution. The solution of the values of the primary slimes is then transferred to container 35 (Fig. 7a) by means of conduit 36. Further amounts of primary slimes are introduced into container 35 by means of channel 37. The primary slimes have an oxidizing effect on ferrous and cuprous ions and an acid neutralizing effect which may be expressed by the following reactions:



- 30 The reaction is complete when the pH rises to pH 4.3 to 4.5. The oxidation reaction is carried out at 180° F. By suitable control it is possible to carry out the reaction to yield a solution of cobalt, nickel, and copper essentially free of iron, 35 and to produce a secondary iron slime containing about 1% to about 2% cobalt, about 2% to about 4% nickel, about 5% to about 7% copper and about 36% to about 40% iron, from 2.5% to 3.5% arsenic and about 0.2% to 0.3% lead.
- 40 The suspension of primary slimes in container 35 is transferred to filter press 38 by any suitable means 39. The fluid portion of the suspension of the primary cobalt-containing iron slimes after separation from the secondary iron slime by any 45 suitable means, such as filter 38, is transferred to container 40 by suitable means 41 and treated with reduced nickel powder in container 40 at a temperature of about 130° F. to about 150° F. and preferably at about 150° F. and at a pH of 4.5 to about 5.5, and preferably at about pH 5.2. Under these conditions, the copper contained in the primary iron slimes and present in the fluid portion as copper sulfate, or chloride, or both, is 55 precipitated out as cement-copper by the addition of the nickel powder. The suspension containing the cement-copper is then transferred by any suitable means 42 to filter press or the like 43 and the cement-copper separated from the fluid portion containing nickel and cobalt as soluble 60 nickel and cobalt sulfates and/or chlorides. The solution containing the nickel and cobalt as soluble salts is then transferred by suitable means 44 to container 45, to which alkaline sodium hypochlorite is added. This hypochlorite solution is 65 made up preferably by chlorinating a soda ash solution containing 3.89 pounds of soda ash per pound of chlorine added. Sufficient hypochlorite solution is added to container 45 so that the cobalt is precipitated as a hydrated cobaltic oxide.
- 70 The residual cobalt content of the solution is reduced to 0.2 gram per liter cobalt by this means. For the precipitation of the cobalt, the temperature of the solution should be maintained at about 80° F. to about 120° F., and preferably at about 100° F. and the pH should be maintained 75

within the range of about pH 1.8 to about pH 2.4 and preferably at about pH 2.3. The precipitated cobalt contains 53 to 55% cobalt and 2% to 4% nickel after the initial separation from the nickel bearing solution. The precipitate formed in tank 48 is allowed to settle, the liquid portion decanted, the precipitate washed once with water, resuspended with water, and redissolved with sulfur dioxide plus sulfuric acid. By suitable control, a solution free from sulfur dioxide at pH 2.0 is obtained. The solution at this point contains approximately 30 grams per liter cobalt and 1 to 2 grams per liter nickel. The cobalt is again precipitated by the action of alkaline sodium hypochlorite to yield a precipitate containing 55% to 57% cobalt and 0.4% to 0.6% nickel, and a solution containing approximately 0.2 gram per liter cobalt and approximately 1 gram per liter nickel. The precipitate is allowed to settle, the fluid portion decanted or separated by any suitable means, and the precipitate washed twice by decantation and finally separated from the wash water by means of filter press 46 into which the suspension is introduced by suitable means 47. The fluid electrolyte, after the initial removal of cobalt to provide a nickel solution containing not more than about 0.2 gram of cobalt per liter, is then transferred by means of channel 48 to tank 49 and treated with soda ash to precipitate the nickel as basic nickel carbonate. This suspension is transferred by suitable means 50 to filter press 51 or the like and the nickel carbonate separated. The precipitate is washed, re-emulsified with water in tank 52 and transferred to oxidation tank 8 by means of conduit 53 to assist in the precipitation of cobalt.

When the primary iron slimes are substantially devoid of cobalt, the treatment to which the primary iron slimes is subjected is somewhat different from that to which primary iron slimes containing cobalt is subjected. This treatment of primary iron slimes substantially devoid of cobalt will be discussed in conjunction with the unit for recovery of nickel from primary iron slimes (Figs. 7 and 7a). The primary iron slimes substantially devoid of cobalt are transferred by means of channel 55 to container 56 (Fig. 7a). Anode slime wash water containing about 3 grams per liter to about 5 grams per liter of chloride ion is introduced into container 56 by means of conduit 57. When desired, anode slime wash water can be added by suitable means 58 to the suspension of the primary iron slimes substantially devoid of cobalt in channel 55 in addition to introducing the anode slime wash water into container 56. The suspension is then conveyed by means of conduit 59 to container 60 where a temperature of about 170° F. to about 180° F. is maintained together with a pH of about 2.0 to about 3.5. Anolyte, from the anode compartments of the electro-refining cells having insoluble anodes, is likewise introduced into container 60 by means of conduit 61. The anolyte so introduced has a pH of about 1.3 to about 1.5 and contains about 0.2 to about 0.4 gram per liter of molecular chlorine. Under these conditions, the major portion of the nickel of the primary iron slimes, together with some arsenic, lead, iron and copper pass into solution. The suspension is conveyed, as by pump 62 and pipe 63, to filter press 64, or any other suitable means, wherein the solids are separated from the fluid portion of the suspension. The fluid portion containing nickel, copper, some iron, arsenic and lead is con-

veyed by conduit 65 to the container 3 and mixed with the impure anolyte therein. The solids are removed and shipped to the copper refinery for separation of the copper and nickel from the iron. These secondary iron slimes contain about 43% to about 45% iron, about 3% to about 4% nickel and about 2% to about 3% copper, 1.5% to 2.0% arsenic and 0.1% to 0.2% lead.

During the corrosion of the impure soluble anodes, the precious metals, gold, silver and the metals of the platinum metal group remain on the corroded anodes as anode slimes. This anode slime is washed off the residual portion of the soluble anodes 66 in tank 67, preferably with impure electrolyte or anolyte in conduit 68, as illustrated in Figs. 7 and 7a (precious metals recovery unit) from which it flows into slime sump 69. The suspension of anode slimes is then transferred by suitable means such as pump 70 and pipe 71 to a holding tank 72 and finally through channel 73 to a means 74 for separating the fluid portion from the solid portion. The fluid portion is returned to the anode slimes suspension sump 69 by means of conduit 75, while the solid portion is conveyed by suitable means 76 to a holding tank 77 where it is suspended in wash water at a temperature of about 140° F. to about 160° F., and preferably about 150° F. The slimes are then transferred by suitable means 78 to a washing filter press 79 and washed therein until the wash water has a chlorine content not greater than about 0.002 gram per liter, and the washed slime a residual chlorine content of 0.1% to 0.2%. This washing operation is quite necessary for the efficient recovery of the precious metals in the anode slimes. In the presence of small amounts of chlorine a relatively large portion of the precious metals is lost in later steps of the purification process. The thoroughly washed primary slimes are then transferred directly to a calciner. The washed filter cake is transferred directly to a calciner 80 by any suitable means 81. The slimes are roasted to reduce the sulfur content to approximately 0.2% and to obtain oxides of the base metals and some of the platinum group metals. The resulting oxide is then charged into an electric anode furnace 82 along with the proper percentage of coke, and the metal is cast in regular anode moulds 83 to form secondary or precious metal anodes. These are returned to the electro-refining cells and are corroded in regular soluble anode cells set aside for the purpose. To prevent loss of slime during corrosion, these anodes are wrapped in closely woven cotton duck. After essentially complete corrosion, the anode scrap, together with the adhering slime, is transferred to the precious metal concentrating plant where the slime is carefully removed from the scrap and treated with acid for the removal of the base metals from gold and the metals of the platinum group. The secondary anode scrap is returned to the electric anode furnace 82 and returns to the electrolytic nickel refinery as secondary anodes.

In carrying out the electro-refining of nickel in accordance with the aforescribed process, it is essential that the pH of electro-deposition be not higher than about pH 5.0 and not lower than about pH 4.0. The amount of iron present in the impure anolyte should be equal to at least about 15 times the sum of the arsenic and lead present in the impure anolyte. The copper present in the impure anolyte should be equal to about 3.0 to about 4.5 times the amount of iron present

in the impure electrolyte and it is desirable to maintain the ratio of nickel to sodium in the electrolyte at not less than 1.50 to 1.00. However, the total sodium present should not exceed 30 grams per liter equivalent to about 75 grams per liter of sodium chloride. In practice it is preferred to maintain the sodium chloride content at about 50 grams per liter. If it is desirable to increase the chloride ion concentration, without further increasing the total sodium ion concentration, it may be accomplished by the addition of calcium chloride to the sulfate-chloride electrolyte followed by filtration to remove the precipitated calcium sulfate. In this manner the chloride ion replaces an equivalent amount of sulfate ion in the solution and there is no increase in the total cation content of the solution. This scheme is used to advantage in changing from an all-sulfate nickel electrolyte having a relatively large concentration of sodium sulfate to a sulfate-chloride nickel electrolyte having a desirable maximum sodium ion concentration of 30 grams per liter. The chlorine necessary for the oxidation of the cobalt is about 2.5 to 3.5 times the theoretical amount. The nickel required for copper cementation is about 1.4 to about 1.5 times the theoretical amount. Nickel required for copper cementation from all-sulfate electrolyte is about 1.9 to about 2 times the theoretical amount. The electrolyte preferably has the following composition:

| Constituents                          | Grams per liter        |
|---------------------------------------|------------------------|
| Nickel.....                           | About 40 to about 60.  |
| Cl <sup>-</sup> .....                 | About 27 to about 30.  |
| SO <sub>4</sub> <sup>2-</sup> .....   | About 71 to about 120. |
| Na <sub>2</sub> SO <sub>4</sub> ..... | About 10 to about 35.  |
| NaCl.....                             | About 45 to about 50.  |
| H <sub>3</sub> BO <sub>3</sub> .....  | About 15 to about 25.  |

The impure anolyte prior to treatment to provide purified electrolyte has the following composition:

| Constituents                          | Grams per liter               |
|---------------------------------------|-------------------------------|
| Nickel.....                           | About 40 to about 60.         |
| Cl <sup>-</sup> .....                 | About 27 to about 30.         |
| SO <sub>4</sub> <sup>2-</sup> .....   | About 71 to about 120.        |
| Na <sub>2</sub> SO <sub>4</sub> ..... | About 10 to about 35.         |
| NaCl.....                             | About 45 to about 50.         |
| H <sub>3</sub> BO <sub>3</sub> .....  | About 15 to about 25.         |
| Cobalt.....                           | About 0.12 to about 0.15.     |
| Iron.....                             | About 0.07 to about 0.10.     |
| Copper.....                           | About 0.25 to about 0.45.     |
| Arsenic.....                          | About 0.004 to about 0.006.   |
| Lead.....                             | About 0.0002 to about 0.0004. |

The purified electrolyte has the following composition:

| Constituents                         | Grams per liter               |
|--------------------------------------|-------------------------------|
| Nickel.....                          | About 40 to about 60.         |
| Sodium.....                          | About 20 to about 30.         |
| Cl <sup>-</sup> .....                | About 27 to about 30.         |
| SO <sub>4</sub> <sup>2-</sup> .....  | About 71 to about 120.        |
| H <sub>3</sub> BO <sub>3</sub> ..... | About 15 to about 25.         |
| Cobalt.....                          | About 0.001 to about 0.01.    |
| Iron.....                            | About 0.0001.                 |
| Copper.....                          | About 0.0002 to about 0.0005. |
| Arsenic.....                         | About 0.0001.                 |
| Lead.....                            | About 0.0001.                 |

The pH of the anolyte in the anode compartments of the cells having soluble anodes should be maintained between a pH of about 4.0 to about 5.0 and preferably at a pH of about 4.5. The pH of the catholyte in the cathode compartments of

the cells employing soluble anodes should be maintained within a range of about pH 4.0 to about pH 5.0. The anolyte in the cells having insoluble anodes should be maintained at about pH 1.25 to about pH 1.5 and preferably at about pH 1.4 and the pH of the catholyte of the cells employing insoluble anodes should be about 4.0 to 5.0 and preferably about pH 4.5. The precipitation of the iron, arsenic and lead without substantial precipitation of the cobalt is carried out at a temperature of about 130° F. to about 135° F. and a pH of about 4.0 to about 4.5, and preferably at a temperature of about 135° F. and a pH of about 4.2. The removal of iron, arsenic and lead together with cobalt is carried out at a temperature of about 130° F. to about 135° F. and preferably at about 135° F. and a pH of about 4.0 to about 5.0 and preferably at about pH 4.5. The removal of copper by cementation is carried out at a temperature of about 130° F. to about 135° F. and preferably at about 135° F. while the pH is allowed to rise from about 4.2 to about 5.4.

When the cobalt present has not been removed simultaneously with the iron, lead and arsenic, it is preferred to carry out the precipitation of the cobalt at a pH of about 4.0 to about 5.0 and a temperature of about 135° F. although satisfactory results can be obtained employing a pH of about 4.0 to about 5.0 and a temperature of about 120° F. to about 180° F.

In the treatment of primary iron slimes containing cobalt, the pH during the reduction of the oxidized slimes to the reduced condition should be allowed to change from pH 6.5 to pH 4.5 by the action of sulfur dioxide. The pH is then reduced to 2.0 by sulfuric acid additions with the temperature of the reaction maintained within the range of 80° F. to about 150° F. and preferably at about 120° F. The reoxidation of the reduced ions of the primary iron slimes should be carried out within a pH range of about 2.0 to about 4.5 and preferably finishing off at about pH 4.5 and at a temperature of about 160° F. to about 180° F. and preferably at about 180° F. The removal of copper by cementation from the primary iron slimes solution should be carried out at a temperature of about 120° F. to about 160° F. and preferably at about 130° F. and within the pH range of about 4.0 to about 5.5 and preferably at about 5.2. It is preferred to maintain a pH of about 2.3 and a temperature of about 100° F. in precipitating the cobalt from the solution derived from the secondary iron slimes. However, this precipitation may be carried out within the range of about pH 1.8 to about pH 2.5 and at a temperature of about 80° F. to about 130° F. The electro-deposition of the nickel from the purified electrolyte is carried out at current densities of up to about 20 amperes per square foot. It will be noted that these current densities are appreciably greater than the current densities generally employed in electro-refining nickel from all-sulfate electrolytes. In this connection it is to be noted particularly that in contrast with the tendency of the electro-nickel to form large berries when current densities in excess of 12 amperes per square foot are employed with an all sulfate ion electrolyte, electro-nickel produced in the sulfate-chloride electrolyte does not tend to produce large berries at even higher current densities for relatively long periods. Consequently, much higher current densities may be employed without encountering the difficulty arising from the tendency for electro-nickel produced in all-sulfate ion electrolytes to produce large berries

which must be broken off at relatively short intervals in order to avoid damage to the canvas diaphragm. Consequently, the sulfate-chloride electrolyte makes it possible to employ much higher current densities with the concurrent treatment of larger quantities of electrolyte and the production of greater amounts of electro-nickel.

In general appearance, the electro-nickel produced from the sulfate-chloride electrolyte is slightly darker and does not have quite the metallic lustre associated with the normal all-sulfate production. Structurally, the nickel is coarser grained as is recognized by comparison of Figs. 9 and 10. From the standpoint of purity, the sulfate-chloride electro-nickel is superior to the all-sulfate ion electro-nickel. For comparison, the following analysis of electro-nickel produced in the all-sulfate electrolyte as compared to the analysis of electro-nickel produced in the sulfate-ion chloride electrolyte in accordance with the process described hereinbefore is provided:

| Constituents | All-sulfate electrolyte, per cent | Sulfate-chloride electrolyte, per cent |
|--------------|-----------------------------------|----------------------------------------|
| Nickel.....  | 99.18 to 99.29.....               | 99.89 to 99.98.....                    |
| Cobalt.....  | 0.70 to 0.80.....                 | 0.10 to 0.01.....                      |
| Copper.....  | 0.003 to 0.005.....               | 0.005 to 0.003.....                    |
| Iron.....    | 0.008 to 0.008.....               | 0.001.....                             |
| Arsenic..... | 0.002 to 0.003.....               | 0.001.....                             |
| Lead.....    | 0.002 to 0.004.....               | 0.001.....                             |

Although the present invention has been described in conjunction with certain preferred embodiments thereof, those skilled in the art will readily recognize that variations and modifications can be made. Such variations and modifications are to be considered within the purview of the specification and the scope of the appended claims.

I claim:

1. A process for electro-refining nickel in an electrolytic cell having an anode compartment and a cathode compartment separated by a porous diaphragm which comprises anodically corroding impure nickel in said anode compartment with an aqueous solution having sulfate ions and chloride ions as the principal anions and containing about 27 grams to about 30 grams per liter of chloride ions, and about 71 to about 120 grams of sulfate ion per liter while maintaining a pH of about 4.0 to about 5.0 to thereby obtain an impure anolyte containing iron, copper, cobalt, arsenic and lead in the reduced state, said copper being present in an amount equal to about 3.0 to about 4.5 times the amount of iron, continuously removing said impure anolyte from said anode compartment, passing air through said impure anolyte to oxidize said copper to the cupric state, the cupric copper reacting with said iron in the reduced state to oxidize substantially all of said iron to the ferric state whereby said iron is hydrolyzed and precipitated without substantial change in said pH of about 4.0 to about 5.0, treating said impure anolyte with sufficient chlorine gas to oxidize and precipitate arsenic and lead, separating said precipitates of iron, arsenic and lead from said impure anolyte to obtain a partially purified anolyte, removing copper from said partially purified anolyte by treatment with nickel powder, separating said nickel powder from said impure anolyte to obtain partially purified electrolyte, passing additional quantities of chlo-

rine gas through said partially purified electrolyte while adding sufficient nickel carbonate to maintain a pH of about 4.0 to about 5.0 whereby said cobalt is oxidized and precipitated, separating said cobalt precipitate from said partially purified electrolyte to obtain purified electrolyte, introducing said purified electrolyte into said cathode compartment, and maintaining a sufficient hydrostatic head in said cathode compartment to substantially prevent the flow of anions from said anode compartment to said cathode compartment.

2. The process as set forth and described in claim 1 in which the copper is precipitated at a pH of about 4.0 to about 5.5.

3. The process as set forth and described in claim 1 wherein the electro-deposition of nickel of high purity is carried out at current densities of about 12 to 20 amperes per square foot.

4. A process for electro-refining nickel which comprises establishing an aqueous solution having a pH of about 4 to about 5 containing about 40 to about 60 grams of nickel per liter, about 20 to about 30 grams of sodium per liter, about 25

27 to about 30 grams of chlorine per liter, about 71 to about 120 grams of sulfate ion per liter, about 15 to about 25 grams of boric acid per liter, not more than 0.01 gram of cobalt per liter, not more than about 0.0001 gram of iron per liter, not more than about 0.0005 gram of copper per liter, not more than about 0.0001 gram of arsenic per liter, and not more than about 0.0001 gram of lead per liter, introducing said electrolyte into the cathode compartment of an electro-

35 depositing cell, said anode compartment being separated from said cathode compartment by a porous diaphragm, electro-depositing nickel at a cathode in said cathode compartment, forcing a portion of said catholyte through said porous diaphragm into said anode compartment under sufficient pressure to substantially prevent copper ions, cobalt ions and ions of other impurities, passing through said diaphragm into said cathode compartment, anodically corroding an impure

40 nickel anode containing copper, iron, cobalt, arsenic and lead, as well as nickel in said electrolyte forced into said anode compartment thereby obtaining a regenerated electrolyte containing increased amounts of nickel and prohibitive amounts of the impurities cobalt, copper, iron, arsenic and lead in the reduced state, said copper being present in an amount equal to about 3.0 to about 4.5 times the amount of iron, said regenerated electrolyte having a pH of about 4 to

45 5 about 5, passing oxygen through said regenerated electrolyte to oxidize said copper to the cupric state, the cupric copper reacting on the said iron in the reduced state to oxidize substantially all of said iron to the ferric state whilst maintaining the aforesaid pH, passing chlorine into said regenerated electrolyte to oxidize said arsenic and lead, allowing sufficient time for the hydrolysis of said oxidized iron salts to obtain a precipitate

50 containing iron, arsenic and lead, separating said precipitate of iron, arsenic and lead from said regenerated electrolyte to obtain a partially purified electrolyte, adding metallic nickel to said partially purified electrolyte to precipitate copper, separating said precipitated copper from said

55 partially purified electrolyte to obtain a further purified electrolyte substantially devoid of iron, copper, arsenic and lead impurities and containing nickel and cobalt, precipitating said cobalt by introducing chlorine and nickel carbonate into

said further purified electrolyte, separating said precipitated cobalt from said further purified electrolyte to obtain a purified electrolyte containing about 40 to about 60 grams of nickel per liter, about 20 to about 30 grams of sodium per liter, about 27 to about 30 grams of chlorine per liter, about 71 to about 120 grams of sulfate ion per liter, about 15 to about 25 grams of boric acid per liter, not more than 0.01 gram of cobalt per liter, not more than about 0.0001 gram of iron per liter, not more than about 0.0005 gram of copper per liter, not more than about 0.0001 gram of arsenic per liter, and not more than about 0.0001 gram of lead per liter, and introducing said purified electrolyte into the cathode compartment of an electro-depositing cell.

5. A process for electro-refining nickel in an electrolytic cell having an anode compartment and a cathode compartment separated by a porous diaphragm which comprises anodically corroding impure nickel in said anode compartment with an aqueous solution comprising essentially about 27 to about 30 grams of chloride ion per liter, about 71 to about 120 grams of sulfate ion per liter, about 20 to about 30 grams of sodium ion per liter, and about 15 to about 25 grams of boric acid per liter while maintaining a pH of about 4.0 to about 5.0 to thereby obtain an impure anolyte containing about 40 to about 60 grams per liter of nickel, about 0.25 to about 0.45 gram per liter of copper, about 0.12 to about 0.15 gram per liter of cobalt, about 0.07 to about 0.10 gram per liter of iron, about 0.0002 to about 0.0004 gram per liter of lead and about 0.004 to about 0.006 gram per liter of arsenic in the reduced state, continuously removing said impure anolyte from said anode compartment, passing air through said impure anolyte to oxidize said copper to the cupric state, the cupric copper reacting with said iron in the reduced state to oxidize substantially all of said iron to the ferric state whereby said iron is hydrolyzed and precipitated without substantial change in said pH of about 4.0 to about 5.0, treating said impure anolyte with sufficient chlorine gas to oxidize and precipitate arsenic and lead, separating said precipitates of iron, arsenic and lead from said impure anolyte to obtain a partially purified anolyte, removing copper from said partially purified anolyte by treatment with nickel powder, separating said nickel powder from said impure anolyte to obtain partially purified electrolyte, passing additional quantities of chlorine gas through said partially purified electrolyte while adding sufficient nickel carbonate to maintain a pH of about 4.0 to about 5.0 whereby said cobalt is oxidized and precipitated, separating said cobalt precipitate from said partially purified electrolyte to obtain purified electrolyte, introducing said purified electrolyte into said cathode compartment, maintaining a sufficient hydrostatic head in said cathode compartment to substantially prevent the flow of anions from said anode compartment to said cathode compartment, and depositing nickel of high purity.

6. A process for electro-refining nickel in an electrolytic cell having an anode compartment and a cathode compartment separated by a porous diaphragm which comprises anodically corroding impure nickel in said anode compartment with an aqueous solution having sulfate ions and chloride ions as the principal anions and containing about 27 grams to about 30 grams per liter of chloride ions and about 71 to about 120

grams of sulfate ion per liter while maintaining a pH of about 4.0 to about 5.0 to thereby obtain an impure anolyte containing iron, copper, cobalt, arsenic and lead in the reduced state, said copper being present in an amount equal to about 3.0 to about 4.5 times the amount of iron, removing said impure anolyte from said anode compartment, passing a relatively weak oxidizing agent comprising oxygen-containing gases through said impure anolyte to oxidize said copper to the cupric state, the cupric copper reacting with said iron in the reduced state to oxidize substantially all of said iron to the ferric state whereby said iron is hydrolyzed and precipitated without substantial change in said pH of about 4 to about 5, oxidizing said reduced arsenic and lead of said impure anolyte to precipitate arsenic and lead, separating said precipitates of iron, arsenic and lead from said impure anolyte to obtain a partially purified anolyte, removing copper from said partially purified anolyte by treatment with nickel powder, separating said nickel powder from said impure anolyte to obtain partially purified electrolyte, adding additional quantities of a relatively strong oxidizing agent to said partially purified electrolyte together with sufficient alkali to maintain a pH of about 4.0 to about 5.0 whereby said cobalt is oxidized and precipitated, separating said cobalt precipitate from said partially purified electrolyte to obtain purified electrolyte, introducing said purified electrolyte into said cathode compartment, and maintaining a sufficient hydrostatic head in said cathode compartment to substantially prevent the flow of anions from said anode compartment to said cathode compartment.

7. A process for electro-refining nickel in an electrolytic cell having an anode compartment and a cathode compartment separated by a porous diaphragm which comprises anodically corroding impure nickel in said anode compartment with an aqueous solution comprising essentially about 27 to about 30 grams of chloride ion per liter, about 71 to about 120 grams of sulfate ion per liter, about 20 to about 30 grams of sodium ion per liter, and about 15 to about 25 grams of boric acid per liter while maintaining a pH of about 4.0 to about 5.0 to thereby obtain an impure anolyte containing about 40 to about 60 grams per liter of nickel, about 0.25 to about 0.45 gram per liter of copper, about 0.12 to about 0.15 gram per liter of cobalt, about 0.07 to about 0.10 gram per liter of iron, about 0.0002 to about 0.0004 gram per liter of lead and about 0.004 to about 0.006 gram per liter of arsenic in the reduced state, continuously removing said impure anolyte from said anode compartment, passing air through said impure anolyte to oxidize said copper to the cupric state, the cupric copper reacting with said iron in the reduced state to oxidize substantially all of said iron to the ferric state whereby said iron is hydrolyzed and precipitated without substantial change in said pH of about 4.0 to about 5.0, treating said impure anolyte with sufficient chlorine gas to oxidize and precipitate arsenic, lead and cobalt while adding enough nickel carbonate to maintain a pH of about 4.0 to about 5.0, separating said precipitates of iron, arsenic, lead and cobalt from said impure anolyte to obtain a partially purified anolyte, removing copper from said partially purified anolyte by successive treatments with nickel powder or progressively increasing purity, separating said nickel powder from said partially purified anolyte

to obtain a purified electrolyte, adjusting the pH of the purified electrolyte to about 4.0 to about 5.0 by addition of acid thereto to obtain a catholyte, introducing said catholyte into said cathode compartment, and maintaining a sufficient hydrostatic head in said cathode compartment to substantially prevent the flow of anions from said anode compartment to said cathode compartment.

8. A process for electro-refining nickel in an electrolytic cell having an anode compartment and a cathode compartment separated by a previous diaphragm which comprises anodically corroding impure nickel in said anode compartment with an aqueous solution having sulfate ions, chloride ions and borate ions as the principal anions and containing about 27 grams to about 30 grams per liter of chloride ions and about 71 to about 120 grams of sulfate ion per liter while maintaining a pH of about 4.0 to about 5.0 to thereby obtain an impure anolyte containing iron, copper, cobalt, arsenic and lead in the reduced state, said copper being present in an amount equal to about 3.0 to about 4.5 times the amount of iron, continuously removing said impure anolyte from said anode compartment, passing air through said impure anolyte to oxidize said copper to the cupric state, the cupric copper reacting with said iron in the reduced state to oxidize substantially all of said iron to the ferric state whereby said iron is hydrolyzed and precipitated without substantial change in said pH of about 4.0 to about 5.0, treating said impure anolyte with sufficient chlorine gas to oxidize and precipitate arsenic, lead and cobalt while adding enough nickel carbonate to maintain a pH of about 4.0 to about 5.0, separating said precipitates of iron, arsenic, lead and cobalt from said impure anolyte to obtain a partially purified anolyte, removing copper from said partially purified anolyte by successive treatments with nickel powder of progressively increasing purity, separating said nickel powder from said partially purified anolyte to obtain a purified electrolyte, adjusting the pH of said purified electrolyte to about 4.0 to about 5.0 by addition of acid thereto to obtain a catholyte, introducing said catholyte into said cathode compartment, and maintaining a sufficient hydrostatic head in said cathode compartment to substantially prevent the flow of anions from said anode compartment to said cathode compartment.

9. In a process for continuously purifying an impure nickel electrolyte comprising an aqueous solution having sulfate ions and chloride ions as the principal anions and containing about 27 to about 30 grams per liter of chloride ions and about 71 to 120 grams of sulfate ion per liter together with nickel, iron, copper, cobalt, arsenic and lead in the reduced state, said copper being present in an amount equal to about 3.0 to about 4.5 times the amount of iron, the improvement which consists in removing iron in said impure electrolyte by passing air through said impure electrolyte to oxidize said reduced copper of the impure electrolyte to the cupric state, the cupric copper reacting with said iron in the reduced state to oxidize substantially all of said iron to the ferric state whereby said iron is hydrolyzed and precipitated within a pH range of about 4.0 to about 5.0 and filtering the solution to remove said iron precipitate.

10. A process for electro-refining nickel in an electrolytic cell having an anode compartment

and a cathode compartment separated by a previous diaphragm which comprises anodically corroding impure nickel in said anode compartment with an aqueous solution having sulfate ions and chloride ions as the principal anions and containing about 27 grams to about 30 grams per liter of chloride ions and about 71 to about 120 grams per liter of sulfate ions while maintaining a pH of about 4.0 to about 5.0 to thereby obtain an impure anolyte containing iron, copper, cobalt, arsenic and lead in the reduced state, said copper being present in an amount equal to about 3.0 to about 4.5 times the amount of iron, removing said impure anolyte from said anode compartment, passing air through said impure anolyte to oxidize said copper to the cupric state, the cupric copper reacting with said iron in the reduced state to oxidize substantially all of said iron to the ferric state whereby said iron is hydrolyzed and precipitated without substantial change in said pH of about 4.0 to 5.0, oxidizing said reduced arsenic, lead and cobalt of said impure anolyte to precipitate arsenic, lead and cobalt, separating said precipitates of iron, arsenic, lead and cobalt from said impure anolyte to obtain a partially purified anolyte, removing copper from said partially purified anolyte by treatment with nickel powder, separating said nickel powder from said partially purified anolyte to obtain a purified electrolyte, introducing said purified electrolyte into said cathode compartment and maintaining a sufficient hydrostatic head in said cathode compartment to substantially prevent the flow of anions from said anode compartment to said cathode compartment.

11. A process for electro-refining nickel in an electrolytic cell having an anode compartment and a cathode compartment separated by a previous diaphragm which comprises anodically corroding impure nickel in said anode compartment with an aqueous solution having sulfate ions and chloride ions as the principal anions and containing about 27 to 30 grams per liter of chloride ions and about 71 to 120 grams per liter of sulfate ion, while maintaining a pH of about 4.0 to about 5.0 to thereby obtain an impure anolyte containing iron, copper, cobalt, arsenic and lead as impurities, said copper being present in an amount equal to about 3.0 to 4.5 times the amount of iron, removing said impure anolyte from said anode compartment, passing air through said impure anolyte to oxidize said copper to the cupric state, the cupric copper reacting with said iron to oxidize substantially all of said iron to the ferric state whereby said iron is hydrolyzed and precipitated without substantial change in said pH of about 4.0 to 5.0, oxidizing said arsenic and lead of the impure anolyte to precipitate arsenic and lead, removing copper from said impure anolyte by treatment with nickel powder, introducing the thus-purified electrolyte into said cathode compartment, and maintaining a sufficient hydrostatic head in said cathode compartment to substantially prevent the flow of anions from said anode compartment to said cathode compartment.

12. A process for electro-refining nickel in an electrolytic cell having an anode compartment and a cathode compartment separated by a previous diaphragm which comprises anodically corroding impure nickel in said anode compartment with an aqueous solution containing about 27 to about 30 grams per liter of chloride ion and about 71 to 120 grams per liter of sulfate ion

to thereby obtain an impure anolyte containing at least about 0.25 gram per liter of copper and at least about 0.07 gram per liter of iron, said copper being present in an amount equal to about 3.0 to about 4.5 times the amount of iron, removing said impure anolyte from said anode compartment, purifying said impure anolyte by passing air through said impure anolyte to oxidize

said copper to the cupric state, the cupric copper reacting with said iron to oxidize substantially all of said iron to the ferric state whereby said iron is hydrolyzed and precipitated while maintaining a pH of about 4.0 to 5.0, and introducing purified anolyte into said cathode compartment.

LOUIS SECONDO RENZONI.